

# United States Patent Office

2,972,544

Patented Feb. 21, 1961

1

2,972,544

## GLASS COMPOSITION

Chikara Hirayama, Murrysville, Pa., assignor to Westinghouse Electric Corporation, East Pittsburgh, Pa., a corporation of Pennsylvania

No Drawing. Filed Oct. 22, 1959, Ser. No. 847,911

2 Claims. (Cl. 106—53)

This invention relates to glass compositions and has for its primary object to provide a new and useful glass having certain special characteristics making it particularly suitable as the major constituent of an electrical insulating medium for high temperature applications.

Glass compositions according to this invention fall within the following ranges of percentage composition by weight, viz: between 20% and 35% PbO, between 20%

5 molten glass of the desired composition in a suitable mold to produce a disc having a diameter of about 1.5 inches and a thickness of about  $\frac{3}{16}$  inch. The discs were ground and polished to a thickness of about 2 millimeters. Each glass disc was provided with suitable electrodes for making the necessary electrical connections for conducting the tests by applying to both surfaces thereof a silver paint comprising finely divided silver particles dispersed in a resinous vehicle. Tests were performed to determine the specific resistance properties of the several glass compositions, the dissipation factor and the dielectric constant. These determinations are set forth in Table II below. Tests were conducted at the various temperatures indicated.

Table II

| Glass Composition | Test Temp.,<br>°C. | Dissipation Factor, 100<br>tan $\delta$ |        |          | Dielectric Constant |        |          | Specific Resistance,<br>ohm-cm. |                      |
|-------------------|--------------------|-----------------------------------------|--------|----------|---------------------|--------|----------|---------------------------------|----------------------|
|                   |                    | 60 cy.                                  | 1 key. | 100 key. | 60 cy.              | 1 key. | 100 key. | 1 Min.                          | 2 Min.               |
| A-----            | 102                | 0.22                                    | 0.13   | 0.56     | 10.9                | 10.8   | 10.9     | $1.9 \times 10^{15}$            | $4.0 \times 10^{15}$ |
|                   | 205                | 0.60                                    | 0.18   | 0.43     | 11.1                | 11.1   | 11.0     | $2.0 \times 10^{13}$            | $2.1 \times 10^{13}$ |
|                   | 305                | 7.30                                    | 1.19   | 0.48     | 11.7                | 11.4   | 11.3     | $7.4 \times 10^{10}$            | $7.4 \times 10^{10}$ |
|                   | 404                | 152                                     | 16.4   | 0.86     | 16.0                | 12.1   | 11.4     | $1.1 \times 10^9$               | $1.1 \times 10^9$    |
|                   | 500                | -----                                   | 186    | 5.54     | -----               | 18.7   | 12.2     | $6.0 \times 10^7$               | $6.2 \times 10^7$    |
| B-----            | 102                | 0.57                                    | 0.13   | 0.38     | 9.8                 | 9.7    | 9.8      | $3.0 \times 10^{16}$            | $1.5 \times 10^{17}$ |
|                   | 205                | 0.50                                    | 0.16   | 0.47     | 10.1                | 10.0   | 9.9      | $1.4 \times 10^{14}$            | $1.4 \times 10^{14}$ |
|                   | 305                | 3.64                                    | 0.63   | 0.49     | 10.4                | 10.2   | 10.2     | $3.0 \times 10^{11}$            | $3.0 \times 10^{11}$ |
|                   | 404                | 59.90                                   | 6.36   | 0.47     | 12.3                | 10.6   | 10.2     | $3.9 \times 10^9$               | $4.0 \times 10^9$    |
|                   | 500                | -----                                   | 88.2   | 2.73     | -----               | 13.1   | 10.8     | $1.7 \times 10^9$               | $1.8 \times 10^9$    |
| C-----            | 102                | 0.17                                    | 0.11   | 0.32     | 10.2                | 10.1   | 10.1     | $3.4 \times 10^{15}$            | $1.1 \times 10^{17}$ |
|                   | 205                | 0.27                                    | 0.16   | 0.33     | 10.3                | 10.2   | 10.2     | $9.1 \times 10^{13}$            | $9.5 \times 10^{13}$ |
|                   | 303                | 2.51                                    | 0.56   | -----    | 10.6                | 10.4   | 10.4     | $2.3 \times 10^{11}$            | $2.3 \times 10^{11}$ |
|                   | 402                | 71.18                                   | 7.85   | 0.45     | 12.8                | 11.0   | 10.6     | $3.8 \times 10^9$               | $3.9 \times 10^9$    |
|                   | 500                | -----                                   | 106    | 3.00     | -----               | 14.0   | 11.0     | $1.2 \times 10^6$               | $1.2 \times 10^6$    |
| D-----            | 102                | 0.28                                    | 0.14   | 0.40     | 9.1                 | 9.0    | 8.9      | $4.0 \times 10^{16}$            | $2.4 \times 10^{17}$ |
|                   | 205                | 0.22                                    | 0.12   | 0.40     | 9.2                 | 9.2    | 9.0      | $9.0 \times 10^{14}$            | $9.9 \times 10^{14}$ |
|                   | 303                | 1.00                                    | 0.35   | 0.36     | 9.5                 | 9.2    | 9.2      | $1.7 \times 10^{12}$            | $1.6 \times 10^{12}$ |
|                   | 402                | 20.66                                   | 2.73   | 0.40     | 10.2                | 9.6    | 9.4      | $1.6 \times 10^{10}$            | $1.6 \times 10^{10}$ |
|                   | 500                | -----                                   | 34.7   | 1.34     | -----               | 10.7   | 9.6      | $5.1 \times 10^9$               | $5.2 \times 10^9$    |

and 30% BaO, between 10% and 20%  $B_2O_3$ , between 5% and 20%  $SiO_2$ , between 4% and 10% CaO, and between 1% and 10%  $Al_2O_3$ . Any remaining ingredients in the glass composition will be in the form of impurities and will be restricted to below about 2%.

Preferred glass compositions fall within the following ranges of percentage composition by weight, viz: between 22% and 32% PbO, between 25% and 30% BaO, between 12% and 20%  $B_2O_3$ , between 8% and 19%  $SiO_2$ , between 5% and 8% CaO, and between 4% and 9%  $Al_2O_3$ .

Four glass compositions, falling within the preferred ranges above given, are set forth in Table I below. The glass compositions are accompanied by their thermal expansion coefficients, sag points, and specific gravities.

For the purposes of this invention, sag point is defined as that temperature at which a filament of the glass, 2 centimeters in length and 0.16 millimeter in cross sectional diameter, will begin to sag under its own weight when heated throughout its entire length.

45 The glass compositions of this invention have particular application as electrical insulating media for high temperature applications. Application of the glass of this invention will usually be made in finely divided form, preferably in admixture with a suitable finely divided electrical insulating refractory material such as silica ( $SiO_2$ ), alumina ( $Al_2O_3$ ), zirconium silicate ( $ZrSiO_4$ ) and the like.

50 To prepare finely divided particles of glass, ingredients in amounts necessary to provide the desired glass composition are placed in a suitable vessel, dry mixed and then heated to a temperature of from about 1000° C. to about 1100° C. at which temperature the ingredients fuse and form a homogeneous molten glass mass. The molten mass of glass is then poured into water and the glass is shattered (the resulting product being known as "frit"). This frit is ball-milled either wet or dry to the desired particle size.

60 The glass compositions of this invention in admixture with electrically insulating refractory materials are particularly suitable for electrical insulating coatings and

Table I

| Glass  | PbO  | $B_2O_3$ | $Al_2O_3$ | BaO  | $SiO_2$ | CaO | Sag Point, °C. | Specific Gravity | Expansion (25-450° C.) (10 <sup>-4</sup> °C.) |
|--------|------|----------|-----------|------|---------|-----|----------------|------------------|-----------------------------------------------|
| A----- | 29.2 | 19.4     | 4.8       | 29.2 | 9.7     | 7.8 | 578            | 4.4              | 9.3                                           |
| B----- | 30.9 | 15.5     | 7.2       | 25.8 | 15.5    | 5.1 | 576            | 4.07             | -----                                         |
| C----- | 27.8 | 13.9     | 4.6       | 27.8 | 18.5    | 7.4 | 586            | 4.05             | 8.8                                           |
| D----- | 22.1 | 17.7     | 8.8       | 26.6 | 17.7    | 7.1 | 597            | 3.73             | -----                                         |

encapsulants that will be satisfactory for use at temperatures up to about 500° C. It will be noted from the sag points set forth in Table I that electrical insulating coatings comprising the glass compositions of this invention will not be adversely affected by the softening of the glass at operating temperatures as high as about 500° C. Furthermore, the glass compositions of this invention, in finely divided form, will fuse and coalesce when heated to temperatures of from about 700° C. to about 750° C. and at these temperatures the glass has sufficient viscosity to flow and to bond together the refractory material and to produce a substantially nonporous insulating medium.

It is to be understood that the above description is illustrative only, and not in limitation of the invention.

I claim as my invention:

1. A glass composition consisting of, by weight, from

20% to 35% PbO, from 10% to 20% B<sub>2</sub>O<sub>3</sub>, from 20% to 30% BaO, from 5% to 20% SiO<sub>2</sub>, from 4% to 10% CaO, and 1% to 10% Al<sub>2</sub>O<sub>3</sub>.

2. A glass composition consisting of, by weight, from 22% to 32% PbO, from 25% to 30% BaO, from 12% to 20% B<sub>2</sub>O<sub>3</sub>, from 8% to 19% SiO<sub>2</sub>, from 5% to 8% CaO, and from 4% to 9% Al<sub>2</sub>O<sub>3</sub>.

#### References Cited in the file of this patent

#### UNITED STATES PATENTS

|           |                |               |
|-----------|----------------|---------------|
| 2,393,450 | Armistead      | Jan. 22, 1946 |
| 2,417,898 | Armistead      | Mar. 25, 1947 |
| 2,431,983 | Bastick et al. | Dec. 2, 1947  |
| 2,702,749 | Hafner         | Feb. 22, 1955 |